



US008828637B2

(12) **United States Patent**  
**Zhou et al.**

(10) **Patent No.:** **US 8,828,637 B2**  
(45) **Date of Patent:** **Sep. 9, 2014**

(54) **TONER COMPOSITIONS**

(71) Applicant: **Xerox Corporation**, Norwalk, CT (US)

(72) Inventors: **Ke Zhou**, Mississauga (CA); **Karen Ann Moffat**, Brantford (CA); **Maria N V McDougall**, Oakville (CA); **Edward G Zwart**, Mississauga (CA); **Paul J Gerroir**, Oakville (CA)

(73) Assignee: **Xerox Corporation**, Norwalk, CT (US)

(\*) Notice: Subject to any disclaimer, the term of this patent is extended or adjusted under 35 U.S.C. 154(b) by 0 days.

(21) Appl. No.: **14/020,808**

(22) Filed: **Sep. 7, 2013**

(65) **Prior Publication Data**

US 2014/0011131 A1 Jan. 9, 2014

**Related U.S. Application Data**

(62) Division of application No. 12/199,115, filed on Aug. 27, 2008, now Pat. No. 8,530,131.

(51) **Int. Cl.**

**G03G 9/087** (2006.01)  
**G03G 9/093** (2006.01)  
**G03G 9/08** (2006.01)

(52) **U.S. Cl.**

CPC ..... **G03G 9/0825** (2013.01); **G03G 9/09328** (2013.01); **G03G 9/09392** (2013.01); **G03G 9/09371** (2013.01); **G03G 9/08793** (2013.01)

USPC ..... **430/109.4**; **430/109.1**; **430/110.2**

(58) **Field of Classification Search**

USPC ..... **430/109.1**, **109.4**, **110.2**  
See application file for complete search history.

(56) **References Cited**

**U.S. PATENT DOCUMENTS**

3,893,932 A \* 7/1975 Azar et al. ..... **430/110.2**  
5,395,723 A 3/1995 Mahabadi et al.  
6,063,827 A \* 5/2000 Sacripante et al. ..... **522/6**  
6,359,105 B1 3/2002 Ianni et al.  
7,425,398 B2 9/2008 Nosella et al.  
2004/0219448 A1 \* 11/2004 Kato et al. ..... **430/108.6**  
2006/0160010 A1 \* 7/2006 Patel et al. ..... **430/109.4**  
2006/0216626 A1 \* 9/2006 Sacripante et al. ..... **430/109.4**  
2006/0275679 A1 \* 12/2006 Ishiyama et al. ..... **430/42**  
2007/0092821 A1 4/2007 Sato et al.

**FOREIGN PATENT DOCUMENTS**

EP 1 772 778 \* 7/2005

\* cited by examiner

*Primary Examiner* — Peter Vajda

(74) *Attorney, Agent, or Firm* — MDIP LLC

(57) **ABSTRACT**

Toner particles are provided which may include a core and a shell, one or both of which may include a polyester gel. The gel in the shell and/or core may prevent a crystalline resin in the core from migrating to the toner surface.

**20 Claims, 1 Drawing Sheet**





FIG. 1



FIG. 2

**1**  
**TONER COMPOSITIONS**

**CROSS-REFERENCE TO RELATED  
APPLICATIONS**

This application is related to co-pending U.S. application Ser. Nos. 12/198,981 and 12/198,999, both filed on Aug. 27, 2008, the entire disclosures of each of which are hereby incorporated by reference in their entirety.

**BACKGROUND**

The present disclosure relates to toners suitable for electrophotographic apparatuses.

Numerous processes are within the purview of those skilled in the art for the preparation of toners. Emulsion aggregation (EA) is one such method. These toners may be formed by aggregating a colorant with a latex polymer formed by emulsion polymerization. For example, U.S. Pat. No. 5,853,943, the disclosure of which is hereby incorporated by reference in its entirety, is directed to a semi-continuous emulsion polymerization process for preparing a latex by first forming a seed polymer. Other examples of emulsion/aggregation/coalescing processes for the preparation of toners are illustrated in U.S. Pat. Nos. 5,403,693, 5,418,108, 5,364,729, and 5,346,797, the disclosures of each of which are hereby incorporated by reference in their entirety. Other processes are disclosed in U.S. Pat. Nos. 5,527,658, 5,585,215, 5,650,255, 5,650,256 and 5,501,935, the disclosures of each of which are hereby incorporated by reference in their entirety.

Polyester EA ultra low melt (ULM) toners have been prepared utilizing amorphous and crystalline polyester resins. While these toners may exhibit excellent fusing properties including crease minimum fixing temperature (NWT) and fusing latitude, peak gloss of these toners may be unacceptably high. Improved toners thus remain desirable.

**SUMMARY**

The present disclosure provides compositions suitable for use in forming toners and methods for their production. In embodiments, a toner of the present disclosure may include a core including at least one amorphous resin, at least one crystalline resin, and one or more optional ingredients such as optional colorants, optional waxes, and combinations thereof, and a shell including at least one amorphous resin such as poly(propoxylated bisphenol co-fumarate), poly(ethoxylated bisphenol co-fumarate), poly(butyloxylated bisphenol co-fumarate), poly(co-propoxylated bisphenol co-ethoxylated bisphenol co-fumarate), poly(1,2-propylene fumarate), poly(propoxylated bisphenol co-maleate), poly(ethoxylated bisphenol co-maleate), poly(butyloxylated bisphenol co-maleate), poly(co-propoxylated bisphenol co-ethoxylated bisphenol co-maleate), poly(1,2-propylene maleate), poly(propoxylated bisphenol co-itaconate), poly(ethoxylated bisphenol co-itaconate), poly(butyloxylated bisphenol co-itaconate), poly(co-propoxylated bisphenol co-ethoxylated bisphenol co-itaconate), poly(1,2-propylene itaconate), and combinations thereof, wherein the amorphous resin in the core, the amorphous resin in the shell, or both, includes a polyester gel.

In other embodiments, a toner of the present disclosure may include a core including at least one amorphous resin, at least one crystalline resin, and one or more optional ingredients such as optional colorants, optional waxes, and combinations thereof; and a shell including a polyester gel including at least one amorphous resin such as poly(propoxylated bisphenol co-fumarate), poly(ethoxylated bisphenol co-fumarate), poly(butyloxylated bisphenol co-fumarate), poly

(co-propoxylated bisphenol co-ethoxylated bisphenol co-fumarate), poly(1,2-propylene fumarate), poly(propoxylated bisphenol co-maleate), poly(ethoxylated bisphenol co-maleate), poly(butyloxylated bisphenol co-maleate), poly(co-propoxylated bisphenol co-ethoxylated bisphenol co-maleate), poly(1,2-propylene maleate), poly(propoxylated bisphenol co-itaconate), poly(ethoxylated bisphenol co-itaconate), poly(butyloxylated bisphenol co-itaconate), poly(co-propoxylated bisphenol co-ethoxylated bisphenol co-itaconate), poly(1,2-propylene itaconate), and combinations thereof, wherein from about 1% by weight about 50% by weight of the polyester gel is crosslinked.

In embodiments, a process of the present disclosure may include contacting at least one amorphous resin with at least one crystalline resin in a dispersion including at least one surfactant; contacting the dispersion with an optional colorant, at least one surfactant, and an optional wax to form small particles; aggregating the small particles; contacting the small particles with a polyester gel latex including at least one amorphous resin such as poly(propoxylated bisphenol co-fumarate), poly(ethoxylated bisphenol co-fumarate), poly(butyloxylated bisphenol co-fumarate), poly(co-propoxylated bisphenol co-ethoxylated bisphenol co-fumarate), poly(1,2-propylene fumarate), poly(propoxylated bisphenol co-maleate), poly(ethoxylated bisphenol co-maleate), poly(butyloxylated bisphenol co-maleate), poly(co-propoxylated bisphenol co-ethoxylated bisphenol co-maleate), poly(1,2-propylene maleate), poly(propoxylated bisphenol co-itaconate), poly(ethoxylated bisphenol co-itaconate), poly(butyloxylated bisphenol co-itaconate), poly(co-propoxylated bisphenol co-ethoxylated bisphenol co-itaconate), poly(1,2-propylene itaconate), and combinations thereof, to form a shell over the small particles; coalescing the small particles possessing the shell to form toner particles; and recovering the toner particles.

**BRIEF DESCRIPTION OF THE DRAWINGS**

Various embodiments of the present disclosure will be described herein below with reference to the figure wherein:

FIG. 1 is a graph comparing the viscosity of a toner of the present disclosure, possessing a polyester gel in the shell, with a control toner; and

FIG. 2 is a graph comparing the charging (in both A-zone and C-zone) of a toner of the present disclosure, possessing a polyester gel in the shell, with a control toner.

**DETAILED DESCRIPTION**

The present disclosure provides toner particles having desirable charging and gloss properties. The toner particles possess a core-shell configuration, with a polyester gel or partially crosslinked polyester in the core, the shell, or both. The gloss of the resulting toner may be reduced by the presence of the cross-linked polyester in the core and/or shell.

**Core Resins**

Any latex resin may be utilized in forming a toner core of the present disclosure. Such resins, in turn, may be made of any suitable monomer. In the event that the core resin is to be crosslinked, any crosslinkable latex resin may be utilized. Suitable monomers useful in forming the resin include, but are not limited to, styrenes, acrylates, methacrylates, butadienes, isoprenes, acrylic acids, methacrylic acids, acrylonitriles, diol, diacid, diamine, diester, mixtures thereof, and the like. Any monomer employed may be selected depending upon the particular polymer to be utilized.

In embodiments, the polymer utilized to form the resin core may be a polyester resin, including the resins described in U.S. Pat. Nos. 6,593,049 and 6,756,176, the disclosures of each of which are hereby incorporated by reference in their

entirety. Suitable resins may also include a mixture of an amorphous polyester resin and a crystalline polyester resin as described in U.S. Pat. No. 6,830,860, the disclosure of which is hereby incorporated by reference in its entirety.

In embodiments, the resin may be a polyester resin formed by reacting a diol with a diacid in the presence of an optional catalyst. For forming a crystalline polyester, suitable organic diols include aliphatic diols with from about 2 to about 36 carbon atoms, such as 1,2-ethanediol, 1,3-propanediol, 1,4-butanediol, 1,5-pentanediol, 1,6-hexanediol, 1,7-heptanediol, 1,8-octanediol, 1,9-nanediol, 1,10-decanediol, 1,12-dodecanediol and the like; alkali sulfo-aliphatic diols such as sodio 2-sulfo-1,2-ethanediol, lithio 2-sulfo-1,2-ethanediol, potassium 2-sulfo-1,2-ethanediol, sodio 2-sulfo-1,3-propanediol, lithio 2-sulfo-1,3-propanediol, potassium 2-sulfo-1,3-propanediol, mixture thereof, and the like. The aliphatic diol may be, for example, selected in an amount of from about 40 to about 60 mole percent, in embodiments from about 42 to about 55 mole percent, in embodiments from about 45 to about 53 mole percent, and the alkali sulfo-aliphatic diol can be selected in an amount of from about 0 to about 10 mole percent, in embodiments from about 1 to about 4 mole percent of the resin.

Examples of organic diacids or diesters including vinyl diacids or vinyl diesters selected for the preparation of the crystalline resins include oxalic acid, succinic acid, glutaric acid, adipic acid, suberic acid, azelaic acid, sebacic acid, fumaric acid, dimethyl fumarate, dimethyl itaconate, cis, 1,4-diacetoxy-2-butene, diethyl fumarate, diethyl maleate, phthalic acid, isophthalic acid, terephthalic acid, naphthalene-2,6-dicarboxylic acid, naphthalene-2,7-dicarboxylic acid, cyclohexane dicarboxylic acid, malonic acid and mesaconic acid, a diester or anhydride thereof; and an alkali sulfo-organic diacid such as the sodio, lithio or potassium salt of dimethyl-5-sulfo-isophthalate, dialkyl-5-sulfo-isophthalate-4-sulfo-1,8-naphthalic anhydride, 4-sulfo-phthalic acid, dimethyl-4-sulfo-phthalate, dialkyl-4-sulfo-phthalate, 4-sulfo-phenyl-3,5-dicarbomethoxybenzene, 6-sulfo-2-naphthyl-3,5-dicarbomethoxybenzene, sulfo-terephthalic acid, dimethyl-sulfo-terephthalate, 5-sulfo-isophthalic acid, dialkyl-sulfo-terephthalate, sulfoethanediol, 2-sulfopropanediol, 2-sulfobutanediol, 3-sulfopentanediol, 2-sulfohexanediol, 3-sulfo-2-methylpentanediol, 2-sulfo-3,3-dimethylpentanediol, sulfo-p-hydroxybenzoic acid, N,N-bis(2-hydroxyethyl)-2-amino ethane sulfonate, or mixtures thereof. The organic diacid may be selected in an amount of, for example, in embodiments from about 40 to about 60 mole percent, in embodiments from about 42 to about 52 mole percent, in embodiments from about 45 to about 50 mole percent, and the alkali sulfo-aliphatic diacid can be selected in an amount of from about 1 to about 10 mole percent of the resin.

Examples of crystalline resins include polyesters, polyamides, polyimides, polyolefins, polyethylene, polybutylene, polyisobutylene, ethylene-propylene copolymers, ethylene-vinyl acetate copolymers, polypropylene, mixtures thereof, and the like. Specific crystalline resins may be polyester based, such as poly(ethylene-adipate), poly(propylene-adipate), poly(butylene-adipate), poly(pentylene-adipate), poly(hexylene-adipate), poly(octylene-adipate), poly(ethylene-succinate), poly(propylene-succinate), poly(butylene-succinate), poly(pentylene-succinate), poly(hexylene-succinate), poly(octylene-succinate), poly(ethylene-sebacate), poly(propylene-sebacate), poly(butylene-sebacate), poly(pentylene-sebacate), poly(hexylene-sebacate), poly(octylene-sebacate), alkali copoly(5-sulfoisophthaloyl)-copoly(ethylene-adipate), alkali copoly(5-sulfoisophthaloyl)-copoly(propylene-adipate), alkali copoly(5-sulfoisophthaloyl)-copoly(butylene-adipate), alkali

copoly), alkali copoly(5-sulfo-isophthaloyl)-copoly(hexylene-adipate), alkali copoly(5-sulfo-isophthaloyl)-copoly(octylene-adipate), alkali copoly(5-sulfo-isophthaloyl)-copoly(ethylene-adipate), alkali copoly(5-sulfo-isophthaloyl)-copoly(5-sulfo-isophthaloyl)-copoly(propylene-adipate), alkali copoly(5-sulfo-isophthaloyl)-copoly(butylene-adipate), alkali copoly(5-sulfo-isophthaloyl)-copoly(pentylene-adipate), alkali copoly(5-sulfo-isophthaloyl)-copoly(hexylene-adipate), alkali copoly(5-sulfo-isophthaloyl)-copoly(octylene-adipate), alkali copoly(5-sulfoisophthaloyl)-copoly(ethylene-succinate), alkali copoly(5-sulfoisophthaloyl)-copoly(propylene-succinate), alkali copoly(5-sulfoisophthaloyl)-copoly(butylene-succinate), alkali copoly(5-sulfoisophthaloyl)-copoly(pentylene-succinate), alkali copoly(5-sulfoisophthaloyl)-copoly(hexylene-succinate), alkali copoly(5-sulfoisophthaloyl)-copoly(octylene-succinate), alkali copoly(5-sulfo-isophthaloyl)-copoly(ethylene-sebacate), alkali copoly(5-sulfo-isophthaloyl)-copoly(propylene-sebacate), alkali copoly(5-sulfo-isophthaloyl)-copoly(butylene-sebacate), alkali copoly(5-sulfo-isophthaloyl)-copoly(pentylene-sebacate), alkali copoly(5-sulfo-isophthaloyl)-copoly(hexylene-sebacate), alkali copoly(5-sulfo-isophthaloyl)-copoly(ethylene-adipate), alkali copoly(5-sulfo-isophthaloyl)-copoly(propylene-adipate), alkali copoly(5-sulfo-isophthaloyl)-copoly(butylene-adipate), alkali copoly(5-sulfo-isophthaloyl)-copoly(pentylene-adipate), alkali copoly(5-sulfo-isophthaloyl)-copoly(hexylene-adipate), poly(octylene-adipate), wherein alkali is a metal like sodium, lithium or potassium. Examples of polyamides include poly(ethylene-adipamide), poly(propylene-adipamide), poly(butylene-adipamide), poly(pentylene-adipamide), poly(hexylene-adipamide), poly(octylene-adipamide), poly(ethylene-succinamide), and poly(propylene-sebacamide). Examples of polyimides include poly(ethylene-adipimide), poly(propylene-adipimide), poly(butylene-adipimide), poly(pentylene-adipimide), poly(hexylene-adipimide), poly(octylene-adipimide), poly(ethylene-succinimide), poly(propylene-succinimide), and poly(butylene-succinimide).

The crystalline resin may be present, for example, in an amount of from about 5 to about 50 percent by weight of the toner components, in embodiments from about 5 to about 35 percent by weight of the toner components. The crystalline resin can possess various melting points of, for example, from about 30° C. to about 120° C., in embodiments from about 50° C. to about 90° C. The crystalline resin may have a number average molecular weight ( $M_n$ ), as measured by gel permeation chromatography (GPC) of, for example, from about 1,000 to about 50,000, in embodiments from about 2,000 to about 25,000, and a weight average molecular weight ( $M_w$ ) of, for example, from about 2,000 to about 100,000, in embodiments from about 3,000 to about 80,000, as determined by Gel Permeation Chromatography using polystyrene standards. The molecular weight distribution ( $M_w/M_n$ ) of the crystalline resin may be, for example, from about 2 to about 6, in embodiments from about 2 to about 4.

Examples of diacid or diesters including vinyl diacids or vinyl diesters selected for the preparation of amorphous polyesters include dicarboxylic acids or diesters such as terephthalic acid, phthalic acid, isophthalic acid, fumaric acid, dimethyl fumarate, dimethyl itaconate, cis, 1,4-diacetoxy-2-butene, diethyl fumarate, diethyl maleate, maleic acid, succinic acid, itaconic acid, succinic acid, succinic anhydride, dodecylsuccinic acid, dodecylsuccinic anhydride, glutaric acid, glutaric anhydride, adipic acid, pimelic acid, suberic acid, azelaic acid, dodecanediacid, dimethyl terephthalate, diethyl terephthalate, dimethylisophthalate, diethylisophthalate, dimethylphthalate, phthalic anhydride, diethylphthalate, dimethylsuccinate, dimethylfumarate, dimethylmaleate, dimethylglutarate, dimethyladipate, dim-

ethyl dodecylsuccinate, and combinations thereof. The organic diacid or diester may be present, for example, in an amount from about 40 to about 60 mole percent of the resin, in embodiments from about 42 to about 52 mole percent of the resin, in embodiments from about 45 to about 50 mole percent of the resin.

Examples of diols utilized in generating the amorphous polyester include 1,2-propanediol, 1,3-propanediol, 1,2-butanediol, 1,3-butanediol, 1,4-butanediol, pentanediol, hexanediol, 2,2-dimethylpropanediol, 2,2,3-trimethylhexanediol, heptanediol, dodecanediol, bis(hydroxyethyl)-bisphenol A, bis(2-hydroxypropyl)-bisphenol A, 1,4-cyclohexanedimethanol, 1,3-cyclohexanedimethanol, xylenedimethanol, cyclohexanediol, diethylene glycol, bis(2-hydroxyethyl) oxide, dipropylene glycol, dibutylene, and combinations thereof. The amount of organic diol selected can vary, and may be present, for example, in an amount from about 40 to about 60 mole percent of the resin, in embodiments from about 42 to about 55 mole percent of the resin, in embodiments from about 45 to about 53 mole percent of the resin.

Polycondensation catalysts which may be utilized for either the crystalline or amorphous polyesters include tetraalkyl titanates, dialkyltin oxides such as dibutyltin oxide, tetraalkyltins such as dibutyltin dilaurate, and dialkyltin oxide hydroxides such as butyltin oxide hydroxide, aluminum alkoxides, alkyl zinc, dialkyl zinc, zinc oxide, stannous oxide, or combinations thereof. Such catalysts may be utilized in amounts of, for example, from about 0.01 mole percent to about 5 mole percent based on the starting diacid or diester used to generate the polyester resin.

In embodiments, suitable amorphous resins include polyesters, polyamides, polyimides, polyolefins, polyethylene, polybutylene, polyisobutylene, ethylene-propylene copolymers, ethylene-vinyl acetate copolymers, polypropylene, combinations thereof, and the like. Examples of amorphous resins which may be utilized include poly(styrene-acrylate) resins, crosslinked, for example, from about 10 percent to about 70 percent, poly(styrene-acrylate) resins, poly(styrene-methacrylate) resins, crosslinked poly(styrene-methacrylate) resins, poly(styrene-butadiene) resins, crosslinked poly(styrene-butadiene) resins, alkali sulfonated-polyester resins, branched alkali sulfonated-polyester resins, alkali sulfonated-polyimide resins, branched alkali sulfonated-polyimide resins, alkali sulfonated poly(styrene-acrylate) resins, crosslinked alkali sulfonated poly(styrene-methacrylate) resins, alkali sulfonated poly(styrene-butadiene) resins, and crosslinked alkali sulfonated poly(styrene-butadiene) resins. Alkali sulfonated polyester resins may be useful in embodiments, such as the metal or alkali salts of copoly(ethylene-terephthalate)-copoly(ethylene-5-sulfo-isophthalate), copoly(propylene-terephthalate)-copoly(propylene-5-sulfo-isophthalate), copoly(di-

ethylene-terephthalate)-copoly(diethylene-5-sulfo-isophthalate), copoly(propylene-diethylene-terephthalate)-copoly(propylene-diethylene-5-sulfoisophthalate), copoly(propylene-butylene-terephthalate)-copoly(propylene-butylene-5-sulfo-isophthalate), copoly(propoxylated bisphenol-A-fumarate)-copoly(propoxylated bisphenol A-5-sulfo-isophthalate), copoly(ethoxylated bisphenol-A-fumarate)-copoly(ethoxylated bisphenol-A-5-sulfo-isophthalate), and copoly(ethoxylated bisphenol-A-5-sulfo-isophthalate), and wherein the alkali metal is, for example, a sodium, lithium or potassium ion.

Examples of other suitable latex resins or polymers which may be utilized include, but are not limited to, poly(styrene-butadiene), poly(methylstyrene-butadiene), poly(methyl methacrylate-butadiene), poly(ethyl methacrylate-butadiene), poly(propyl methacrylate-butadiene), poly(butyl methacrylate-butadiene), poly(methyl acrylate-butadiene), poly(ethyl acrylate-butadiene), poly(propyl acrylate-butadiene), poly(butyl acrylate-butadiene), poly(styrene-isoprene), poly(methylstyrene-isoprene), poly(methyl methacrylate-isoprene), poly(ethyl methacrylate-isoprene), poly(propyl methacrylate-isoprene), poly(butyl methacrylate-isoprene), poly(methyl acrylate-isoprene), poly(ethyl acrylate-isoprene), poly(propyl acrylate-isoprene), poly(butyl acrylate-isoprene); poly(styrene-propyl acrylate), poly(styrene-butyl acrylate), poly(styrene-butadiene-acrylic acid), poly(styrene-butadiene-methacrylic acid), poly(styrene-butadiene-acrylonitrile-acrylic acid), poly(styrene-butyl acrylate-acrylonitrile), and poly(styrene-butyl acrylate-acrylonitrile-acrylic acid), and combinations thereof. The polymer may be block, random, or alternating copolymers.

In embodiments, an unsaturated polyester resin may be utilized as a latex resin. Examples of such resins include those disclosed in U.S. Pat. No. 6,063,827, the disclosure of which is hereby incorporated by reference in its entirety. Exemplary unsaturated polyester resins include, but are not limited to, poly(propoxylated bisphenol co-fumarate), poly(ethoxylated bisphenol co-fumarate), poly(butyloxylated bisphenol co-fumarate), poly(co-propoxylated bisphenol co-ethoxylated bisphenol co-fumarate), poly(1,2-propylene fumarate), poly(propoxylated bisphenol co-maleate), poly(ethoxylated bisphenol co-maleate), poly(butyloxylated bisphenol co-maleate), poly(co-propoxylated bisphenol co-ethoxylated bisphenol co-maleate), poly(1,2-propylene maleate), poly(propoxylated bisphenol co-itaconate), poly(ethoxylated bisphenol co-itaconate), poly(butyloxylated bisphenol co-itaconate), poly(co-propoxylated bisphenol co-ethoxylated bisphenol co-itaconate), poly(1,2-propylene itaconate), and combinations thereof.

In embodiments, a suitable polyester resin may be an amorphous polyester such as a poly(propoxylated bisphenol A co-fumarate) resin having the following formula (I):



wherein m may be from about 5 to about 1000.

An example of a linear propoxylated bisphenol A fumarate resin which may be utilized as a latex resin is available under the trade name SPARII from Resana S/A Industrias Quimicas, Sao Paulo Brazil. Other propoxylated bisphenol A fumarate resins that may be utilized and are commercially available include GTUF and FPESL-2 from Kao Corporation, Japan, and EM181635 from Reichhold, Research Triangle Park, North Carolina and the like.

Suitable crystalline resins include those disclosed in U.S. Patent Application Publication No. 2006/0222991, the disclosure of which is hereby incorporated by reference in its entirety. In embodiments, a suitable crystalline resin may include a resin composed of ethylene glycol and a mixture of dodecanedioic acid and fumaric acid co-monomers with the following formula:



wherein b is from 5 to 2000 and d is from 5 to 2000.

For example, in embodiments, a poly(propoxylated bisphenol A co-fumarate) resin of formula I as described above may be combined with a crystalline resin of formula II to form a core.

In embodiments, a resin utilized for forming the core may be partially crosslinked, which may be referred to, in embodiments, as a "partially crosslinked polyester resin" or a "polyester gel". In embodiments, from about 1% by weight to about 50% by weight of the polyester gel may be crosslinked, in embodiments from about 5% by weight to about 35% by weight of the polyester gel may be crosslinked.

In embodiments, the amorphous resins described above may be partially crosslinked to form a core. For example, an amorphous resin which may be crosslinked and used in forming a toner particle in accordance with the present disclosure may include a crosslinked amorphous polyester of formula I above. Methods for forming the polyester gel include those within the purview of those skilled in the art. For example, crosslinking may be achieved by combining an amorphous resin with a crosslinker, sometimes referred to herein, in embodiments, as an initiator. Examples of suitable crosslinkers include, but are not limited to, for example, free radical or thermal initiators such as organic peroxides and azo compounds. Examples of suitable organic peroxides include diaryl peroxides such as, for example, decanoyl peroxide, lauroyl peroxide and benzoyl peroxide, ketone peroxides such as, for example, cyclohexanone peroxide and methyl ethyl ketone, alkyl peroxyesters such as, for example, t-butyl peroxy neodecanoate, 2,5-dimethyl 2,5-di(2-ethyl hexanoyl peroxy) hexane, t-amyl peroxy 2-ethyl hexanoate, t-butyl peroxy 2-ethyl hexanoate, t-butyl peroxy acetate, t-amyl peroxy acetate, t-butyl peroxy benzoate, t-amyl peroxy benzoate, oo-t-butyl o-isopropyl mono peroxy carbonate, 2,5-dimethyl 2,5-di(benzoyl peroxy) hexane, oo-t-butyl o-(2-ethyl hexyl) mono peroxy carbonate, and oo-t-amyl o-(2-ethyl hexyl) mono peroxy carbonate, alkyl peroxides such as, for example, dicumyl peroxide, 2,5-dimethyl 2,5-di(t-butyl peroxy) hexane, t-butyl cumyl peroxide,  $\alpha$ - $\alpha$ -bis(t-butyl peroxy)diisopropyl benzene, di-t-butyl peroxide and 2,5-dimethyl 2,5-di(t-butyl peroxy) hexyne-3, alkyl hydroperoxides such as, for

example, 2,5-dihydro peroxy 2,5-dimethyl hexane, cumene hydroperoxide, t-butyl hydroperoxide and t-amyl hydroperoxide, and alkyl peroxyketals such as, for example, n-butyl 4,4-di(t-butyl peroxy) valerate, 1,1-di(t-butyl peroxy) 3,3,5-trimethyl cyclohexane, 1,1-di(t-butyl peroxy)cyclohexane, 1,1-di(t-amyl peroxy)cyclohexane, 2,2-di(t-butyl peroxy) butane, ethyl 3,3-di(t-butyl peroxy) butyrate and ethyl 3,3-di(t-amyl peroxy) butyrate, and combinations thereof. Examples of suitable azo compounds include 2,2'-azobis(2,4-dimethylpentane nitrile), azobis-isobutyronitrile, 2,2'-azobis(isobutyronitrile), 2,2'-azobis(2,4-dimethyl valeronitrile), 2,2'-azobis(methyl butyronitrile), 1,1'-azobis(cyano cyclohexane), other similar known compounds, and combinations thereof.

Although any suitable initiator can be used, in embodiments the initiator may be an organic initiator that is soluble in any solvent present, but not soluble in water. For example, half-life/temperature characteristic plots for VAZO® 52 (2,2'-azobis(2,4-dimethylpentane nitrile), commercially available from E. I. du Pont de Nemours and Company, USA) shows a half-life greater than about 90 minutes at about 65°C. and less than about 20 minutes at about 80°C.

Where utilized, the crosslinker may be present in an amount of from about 0.5% by weight to about 20% by weight of the resin, in embodiments from about 1% by weight to about 10% by weight of the resin.

The crosslinker and amorphous resin may be combined for a sufficient time and at a sufficient temperature to form the crosslinked polyester gel. In embodiments, the crosslinker and amorphous resin may be heated to a temperature of from about 25°C. to about 99°C., in embodiments from about 40°C. to about 95°C., for a period of time of from about 1 minute to about 10 hours, in embodiments from about 5 minutes to about 5 hours, to form a crosslinked polyester resin or polyester gel suitable for use in forming toner particles.

In embodiments, the combined amorphous resins utilized in the core may have a glass transition temperature of from about 30°C. to about 80°C., in embodiments from about 35°C. to about 70°C. In further embodiments, the combined resins utilized in the core may have a melt viscosity of from about 10 to about 1,000,000 Pa\*S at about 130°C., in embodiments from about 20 to about 100,000 Pa\*S.

One, two, or more toner resins may be used. In embodiments where two or more toner resins are used, the toner resins may be in any suitable ratio (e.g., weight ratio) such as for instance about 10% (first resin)/90% (second resin) to about 90% (first resin)/10% (second resin).

In embodiments, the resin may be formed by emulsion polymerization methods.

#### Toner

The resin described above may be utilized to form toner compositions. Such toner compositions may include optional colorants, waxes, and other additives. Toners may be formed utilizing any method within the purview of those skilled in the art.

#### Surfactants

In embodiments, colorants, waxes, and other additives utilized to form toner compositions may be in dispersions including surfactants. Moreover, toner particles may be formed by emulsion aggregation methods where the resin and other components of the toner are placed in one or more surfactants, an emulsion is formed, toner particles are aggregated, coalesced, optionally washed and dried, and recovered.

One, two, or more surfactants may be utilized. The surfactants may be selected from ionic surfactants and nonionic surfactants. Anionic surfactants and cationic surfactants are encompassed by the term "ionic surfactants." In embodi-

ments, the surfactant may be utilized so that it is present in an amount of from about 0.01% to about 5% by weight of the toner composition, for example from about 0.75% to about 4% by weight of the toner composition, in embodiments from about 1% to about 3% by weight of the toner composition.

Examples of nonionic surfactants that can be utilized include, for example, polyacrylic acid, methalose, methyl cellulose, ethyl cellulose, propyl cellulose, hydroxy ethyl cellulose, carboxy methyl cellulose, polyoxyethylene cetyl ether, polyoxyethylene lauryl ether, polyoxyethylene octyl ether, polyoxyethylene octylphenyl ether, polyoxyethylene oleyl ether, polyoxyethylene sorbitan monolaurate, polyoxyethylene stearyl ether, polyoxyethylene nonylphenyl ether, dialkylphenoxy poly(ethyleneoxy)ethanol, available from Rhone-Poulenc as IGEPAL CA-210<sup>TM</sup>, IGEPAL CA-520<sup>TM</sup>, IGEPAL CA-720<sup>TM</sup>, IGEPAL CO-890<sup>TM</sup>, IGEPAL CO-720<sup>TM</sup>, IGEPAL CO-290<sup>TM</sup>, IGEPAL CA-21<sup>TM</sup>, ANTAROX 890<sup>TM</sup> and ANTAROX 897<sup>TM</sup>. Other examples of suitable nonionic surfactants include a block copolymer of polyethylene oxide and polypropylene oxide, including those commercially available as SYNPERONIC PE/F, in embodiments SYNPERONIC PE/F 108.

Anionic surfactants which may be utilized include sulfates and sulfonates, sodium dodecylsulfate (SDS), sodium dodecylbenzene sulfonate, sodium dodecylnaphthalene sulfate, dialkyl benzenealkyl sulfates and sulfonates, acids such as abitic acid available from Aldrich, NEOGEN R<sup>TM</sup>, NEOGEN SC<sup>TM</sup> obtained from Daiichi Kogyo Seiyaku, combinations thereof, and the like. Other suitable anionic surfactants include, in embodiments, DOWFAX<sup>TM</sup> 2A1, an alkylidiphenyloxide disulfonate from The Dow Chemical Company, and/or TAYCA POWER BN2060 from Tayca Corporation (Japan), which are branched sodium dodecyl benzene sulfonates. Combinations of these surfactants and any of the foregoing anionic surfactants may be utilized in embodiments.

Examples of the cationic surfactants, which are usually positively charged, include, for example, alkylbenzyl dimethyl ammonium chloride, dialkyl benzenealkyl ammonium chloride, lauryl trimethyl ammonium chloride, alkylbenzyl methyl ammonium chloride, alkyl benzyl dimethyl ammonium bromide, benzalkonium chloride, cetyl pyridinium bromide, C<sub>12</sub>, C<sub>15</sub>, C<sub>17</sub> trimethyl ammonium bromides, halide salts of quaternized polyoxyethylalkylamines, dodecylbenzyl triethyl ammonium chloride, MIRAPOL<sup>TM</sup> and ALKAQUATT<sup>TM</sup>, available from Alkaril Chemical Company, SANIZOL<sup>TM</sup> (benzalkonium chloride), available from Kao Chemicals, and the like, and mixtures thereof.

#### Colorants

As the colorant to be added, various known suitable colorants, such as dyes, pigments, mixtures of dyes, mixtures of pigments, mixtures of dyes and pigments, and the like, may be included in the toner. The colorant may be included in the toner in an amount of, for example, about 0.1 to about 35 percent by weight of the toner, or from about 1 to about 15 weight percent of the toner, or from about 3 to about 10 percent by weight of the toner.

As examples of suitable colorants, mention may be made of carbon black like REGAL 330<sup>®</sup>; magnetites, such as Mobay magnetites MO8029<sup>TM</sup>, MO8060<sup>TM</sup>; Columbian magnetites; MAPICO BLACK<sup>TM</sup> and surface treated magnetites; Pfizer magnetites CB4799<sup>TM</sup>, CB5300<sup>TM</sup>, CB5600<sup>TM</sup>, MCX6369<sup>TM</sup>; Bayer magnetites, BAYFERROX 8600<sup>TM</sup>, 8610<sup>TM</sup>; Northern Pigments magnetites, NP-604<sup>TM</sup>, NP-608<sup>TM</sup>; Magnox magnetites TMB-100<sup>TM</sup>, or TMB-104<sup>TM</sup>; and the like. As colored pigments, there can be selected cyan, magenta, yellow, red, green, brown, blue or

mixtures thereof. Generally, cyan, magenta, or yellow pigments or dyes, or mixtures thereof, are used. The pigment or pigments are generally used as water based pigment dispersions.

- 5 Specific examples of pigments include SUNSPERSE 6000, FLEXIVERSE and AQUATONE water based pigment dispersions from SUN Chemicals, HELIOGEN BLUE L6900<sup>TM</sup>, D6840<sup>TM</sup>, D7080<sup>TM</sup>, D7020<sup>TM</sup>, PYLAM OIL BLUE<sup>TM</sup>, PYLAM OIL YELLOW<sup>TM</sup>, PIGMENT BLUE 1<sup>TM</sup> 10 available from Paul Uhlrich & Company, Inc., PIGMENT VIOLET 1<sup>TM</sup>, PIGMENT RED 48<sup>TM</sup>, LEMON CHROME YELLOW DCC 1026<sup>TM</sup>, E.D. TOLUIDINE RED<sup>TM</sup> and BON RED C<sup>TM</sup> available from Dominion Color Corporation, Ltd., Toronto, Ontario, NOVAPERM YELLOW FGL<sup>TM</sup>, 15 HOSTAPERM PINK E<sup>TM</sup> from Hoechst, and CINQUASIA MAGENTA<sup>TM</sup> available from E.I. DuPont de Nemours & Company, and the like. Generally, colorants that can be selected are black, cyan, magenta, or yellow, and mixtures thereof. Examples of magentas are 2,9-dimethyl-substituted 20 quinacridone and anthraquinone dye identified in the Color Index as CI 60710, CI Dispersed Red 15, diazo dye identified in the Color Index as CI 26050, CI Solvent Red 19, and the like. Illustrative examples of cyans include copper tetra(octadecyl sulfonamido) phthalocyanine, x-copper phthalocyanine pigment listed in the Color Index as CI 74160, CI Pigment Blue, Pigment Blue 15:3, and Anthrathrene Blue, identified in the Color Index as CI 69810, Special Blue X-2137, and the like. Illustrative examples of yellows are diarylide yellow 3,3-dichlorobenzidine acetoacetanilides, a 25 monoazo pigment identified in the Color Index as CI 12700, CI Solvent Yellow 16, a nitrophenyl amine sulfonamide identified in the Color Index as Foron Yellow SE/GLN, CI Dispersed Yellow 33 2,5-dimethoxy-4-sulfonanilide phenylazo-4'-chloro-2,5-dimethoxy acetoacetanilide, and Permanent 30 Yellow FGL. Colored magnetites, such as mixtures of MAPICO BLACK<sup>TM</sup>, and cyan components may also be selected as colorants. Other known colorants can be selected, such as Levanyl Black A-SF (Miles, Bayer) and Sunperse Carbon Black LHD 9303 (Sun Chemicals), and colored dyes 35 such as Neopen Blue (BASF), Sudan Blue OS (BASF), PV Fast Blue B2G01 (American Hoechst), Sunperse Blue BHD 6000 (Sun Chemicals), Irgalite Blue BCA (Ciba-Geigy), Paliogen Blue 6470 (BASF), Sudan III (Matheson, Coleman, Bell), Sudan II (Matheson, Coleman, Bell), Sudan IV (Matheson, Coleman, Bell), Sudan Orange G (Aldrich), Sudan Orange 220 (BASF), Paliogen Orange 3040 (BASF), Ortho Orange OR 2673 (Paul Uhlrich), Paliogen Yellow 152, 45 1560 (BASF), Lithol Fast Yellow 0991K (BASF), Paliotol Yellow 1840 (BASF), Neopen Yellow (BASF), Novoperm Yellow FG 1 (Hoechst), Permanent Yellow YE 0305 (Paul Uhlrich), Lumogen Yellow D0790 (BASF), Sunperse Yellow YHD 6001 (Sun Chemicals), Suco-Gelb L1250 (BASF), Suco-Yellow DI 355 (BASF), Hostaperm Pink E (American Hoechst), Fanal Pink D4830 (BASF), Cinquasia Magenta 50 (DuPont), Lithol Scarlet D3700 (BASF), Toluidine Red (Aldrich), Scarlet for Thermoplast NSD PS PA (Ugine Kuhlmann of Canada), E.D. Toluidine Red (Aldrich), Lithol Rubine Toner (Paul Uhlrich), Lithol Scarlet 4440 (BASF), Bon Red C (Dominion Color Company), Royal Brilliant Red RD-8192 55 (Paul Uhlrich), Oracet Pink RF (Ciba-Geigy), Paliogen Red 3871K (BASF), Paliogen Red 3340 (BASF), Lithol Fast Scarlet L4300 (BASF), combinations of the foregoing, and the like.
- 60 Wax
- 65 Optionally, a wax may also be combined with the resin and optional colorant in forming toner particles. When included, the wax may be present in an amount of, for example, from

## 11

about 1 weight percent to about 25 weight percent of the toner particles, in embodiments from about 5 weight percent to about 20 weight percent of the toner particles.

Waxes that may be selected include waxes having, for example, a weight average molecular weight of from about 500 to about 20,000, in embodiments from about 1,000 to about 10,000. Waxes that may be used include, for example, polyolefins such as polyethylene, polypropylene, and polybutene waxes such as commercially available from Allied Chemical and Petrolite Corporation, for example POLY-WAX<sup>TM</sup> polyethylene waxes from Baker Petrolite, wax emulsions available from Michaelman, Inc. and the Daniels Products Company, EPOLENE N-15<sup>TM</sup> commercially available from Eastman Chemical Products, Inc., and VISCOL 550-P<sup>TM</sup>, a low weight average molecular weight polypropylene available from Sanyo Kasei K. K.; plant-based waxes, such as carnauba wax, rice wax, candelilla wax, sumacs wax, and jojoba oil; animal-based waxes, such as beeswax; mineral-based waxes and petroleum-based waxes, such as montan wax, ozokerite, ceresin, paraffin wax, microcrystalline wax, and Fischer-Tropsch wax; ester waxes obtained from higher fatty acid and higher alcohol, such as stearyl stearate and behenyl behenate; ester waxes obtained from higher fatty acid and monovalent or multivalent lower alcohol, such as butyl stearate, propyl oleate, glyceride monostearate, glyceride distearate, and pentaerythritol tetra behenate; ester waxes obtained from higher fatty acid and multivalent alcohol multimers, such as diethyleneglycol monostearate, dipropylene-glycol distearate, diglyceryl distearate, and triglyceryl tetra stearate; sorbitan higher fatty acid ester waxes, such as sorbitan monostearate, and cholesterol higher fatty acid ester waxes, such as cholesteryl stearate. Examples of functionalized waxes that may be used include, for example, amines, amides, for example AQUA SUPERSLIP 6550<sup>TM</sup>, SUPER-SLIP 6530<sup>TM</sup> available from Micro Powder Inc., fluorinated waxes, for example POLYFLUO 190<sup>TM</sup>, POLYFLUO 200<sup>TM</sup>, POLYSILK 19<sup>TM</sup>, POLYSILK 14<sup>TM</sup> available from Micro Powder Inc., mixed fluorinated, amide waxes, for example MICROSPERSION 19<sup>TM</sup> also available from Micro Powder Inc., imides, esters, quaternary amines, carboxylic acids or acrylic polymer emulsion, for example JONCRYL 74<sup>TM</sup>, 89<sup>TM</sup>, 130<sup>TM</sup>, 537<sup>TM</sup>, and 538<sup>TM</sup>, all available from SC Johnson Wax, and chlorinated polypropylenes and polyethylenes available from Allied Chemical and Petrolite Corporation and SC Johnson wax. Mixtures and combinations of the foregoing waxes may also be used in embodiments. Waxes may be included as, for example, fuser roll release agents.

## Toner Preparation

The toner particles may be prepared by any method within the purview of one skilled in the art. Although embodiments relating to toner particle production are described below with respect to emulsion-aggregation processes, any suitable method of preparing toner particles may be used, including chemical processes, such as suspension and encapsulation processes disclosed in U.S. Pat. Nos. 5,290,654 and 5,302,486, the disclosures of each of which are hereby incorporated by reference in their entirety. In embodiments, toner compositions and toner particles may be prepared by aggregation and coalescence processes in which small-size resin particles are aggregated to the appropriate toner particle size and then coalesced to achieve the final toner particle shape and morphology.

In embodiments, toner compositions may be prepared by emulsion-aggregation processes, such as a process that includes aggregating a mixture of an optional colorant, an optional wax and any other desired or required additives, and

## 12

emulsions including the resins described above, optionally in surfactants as described above, and then coalescing the aggregate mixture. A mixture may be prepared by adding a colorant and optionally a wax or other materials, which may also be 5 optionally in a dispersion(s) including a surfactant, to the emulsion, which may be a mixture of two or more emulsions containing the resin. The pH of the resulting mixture may be 10 adjusted by an acid such as, for example, acetic acid, nitric acid or the like. In embodiments, the pH of the mixture may 15 be adjusted to from about 4 to about 5. Additionally, in embodiments, the mixture may be homogenized. If the mixture is homogenized, homogenization may be accomplished by mixing at about 600 to about 4,000 revolutions per minute. Homogenization may be accomplished by any suitable 20 means, including, for example, an IKA ULTRA TURRAX T50 probe homogenizer.

Following the preparation of the above mixture, an aggregating agent may be added to the mixture. Any suitable aggregating agent may be utilized to form a toner. Suitable aggregating agents include, for example, aqueous solutions of a 25 divalent cation or a multivalent cation material. The aggregating agent may be, for example, polyaluminum halides such as polyaluminum chloride (PAC), or the corresponding bromide, fluoride, or iodide, polyaluminum silicates such as 30 polyaluminum sulfosilicate (PASS), and water soluble metal salts including aluminum chloride, aluminum nitrite, aluminum sulfate, potassium aluminum sulfate, calcium acetate, calcium chloride, calcium nitrite, calcium oxylate, calcium sulfate, magnesium acetate, magnesium nitrate, magnesium sulfate, zinc acetate, zinc nitrate, zinc sulfate, zinc chloride, zinc bromide, magnesium bromide, copper chloride, copper sulfate, and combinations thereof. In embodiments, the aggregating agent may be added to the mixture at a temperature that is below the glass transition temperature (Tg) of the 35 resin.

The aggregating agent may be added to the mixture utilized to form a toner in an amount of, for example, from about 0.1% to about 8% by weight, in embodiments from about 0.2% to about 5% by weight, in other embodiments from about 0.5% 40 to about 5% by weight, of the resin in the mixture. This provides a sufficient amount of agent for aggregation.

In order to control aggregation and subsequent coalescence of the particles, in embodiments the aggregating agent may be metered into the mixture over time. For example, the agent 45 may be metered into the mixture over a period of from about 5 to about 240 minutes, in embodiments from about 30 to about 200 minutes, although more or less time may be used as desired or required. The addition of the agent may also be done while the mixture is maintained under stirred conditions, in embodiments from about 50 rpm to about 1,000 rpm, in other embodiments from about 100 rpm to about 500 rpm, and at a temperature that is below the glass transition temperature of the resin as discussed above, in embodiments from about 30° C. to about 90° C., in embodiments from 55 about 35° C. to about 70° C.

The particles may be permitted to aggregate until a predetermined desired particle size is obtained. A predetermined desired size refers to the desired particle size to be obtained as determined prior to formation, and the particle size being 60 monitored during the growth process until such particle size is reached. Samples may be taken during the growth process and analyzed, for example with a Coulter Counter, for average particle size. The aggregation thus may proceed by maintaining the elevated temperature, or slowly raising the temperature to, for example, from about 30° C. to about 99° C., and holding the mixture at this temperature for a time from about 65 0.5 hours to about 10 hours, in embodiments from about hour

## 13

1 to about 5 hours, while maintaining stirring, to provide the aggregated particles. Once the predetermined desired particle size is reached, then the growth process is halted. In embodiments, the predetermined desired particle size is within the toner particle size ranges mentioned above.

The growth and shaping of the particles following addition of the aggregation agent may be accomplished under any suitable conditions. For example, the growth and shaping may be conducted under conditions in which aggregation occurs separate from coalescence. For separate aggregation and coalescence stages, the aggregation process may be conducted under shearing conditions at an elevated temperature, for example of from about 40° C. to about 90° C., in embodiments from about 45° C. to about 80° C., which may be below the glass transition temperature of the resin as discussed above.

Once the desired final size of the toner particles is achieved, the pH of the mixture may be adjusted with a base to a value of from about 3 to about 10, and in embodiments from about 5 to about 9. The adjustment of the pH may be utilized to freeze, that is to stop, toner growth. The base utilized to stop toner growth may include any suitable base such as, for example, alkali metal hydroxides such as, for example, sodium hydroxide, potassium hydroxide, ammonium hydroxide, combinations thereof, and the like. In embodiments, ethylene diamine tetraacetic acid (EDTA) may be added to help adjust the pH to the desired values noted above.

## Shell Resin

In embodiments, after aggregation, but prior to coalescence, a shell may be applied to the aggregated particles. In embodiments, a resin utilized for forming the shell may be partially crosslinked, which may be referred to, in embodiments, as a "partially crosslinked polyester resin" or a "polyester gel". The crosslinked portion of the gel can be determined by any suitable method within the purview of those skilled in the art, for example, the gel can be dissolved in a suitable solvent, such as, toluene, then the weight of the insolubles may be measured.

In embodiments, from about 1% by weight to about 50% by weight of the shell resin may be crosslinked, in embodiments from about 5% by weight to about 35% by weight of the shell resin may be crosslinked.

Resins which may be utilized to form a polyester gel as a shell include, but are not limited to, the amorphous resins described above for use in the core. In embodiments, an amorphous resin which may be crosslinked and used as a polyester gel to form a shell in accordance with the present disclosure may include a crosslinked amorphous polyester of formula I above. Methods for forming the polyester gel include those within the purview of those skilled in the art. For example, crosslinking may be achieved by combining an amorphous resin with a crosslinker, sometimes referred to herein, in embodiments, as an initiator. Examples of suitable crosslinkers include, but are not limited to, for example free radical or thermal initiators such as organic peroxides and azo compounds described above as suitable for forming a gel in the core. Examples of suitable organic peroxides include diacyl peroxides such as, for example, decanoyl peroxide, lauroyl peroxide and benzoyl peroxide, ketone peroxides such as, for example, cyclohexanone peroxide and methyl ethyl ketone, alkyl peroxyesters such as, for example, t-butyl peroxy neodecanoate, 2,5-dimethyl 2,5-di(2-ethyl hexanoyl peroxy) hexane, t-amyl peroxy 2-ethyl hexanoate, t-butyl peroxy 2-ethyl hexanoate, t-butyl peroxy acetate, t-amyl peroxy acetate, t-butyl peroxy benzoate, t-amyl peroxy benzoate, oo-t-butyl o-isopropyl mono peroxy carbonate, 2,5-dimethyl 2,5-di(benzoyl peroxy) hexane, oo-t-butyl o-(2-ethyl hexyl)

## 14

mono peroxy carbonate, and oo-t-amyl o-(2-ethyl hexyl) mono peroxy carbonate, alkyl peroxides such as, for example, dicumyl peroxide, 2,5-dimethyl 2,5-di(t-butyl peroxy) hexane, t-butyl cumyl peroxide,  $\alpha$ - $\alpha$ -bis(t-butyl peroxy)diisopropyl benzene, di-t-butyl peroxide and 2,5-dimethyl 2,5-di(t-butyl peroxy) hexyne-3, alkyl hydroperoxides such as, for example, 2,5-dihydro peroxy 2,5-dimethyl hexane, cumene hydroperoxide, t-butyl hydroperoxide and t-amyl hydroperoxide, and alkyl peroxyketals such as, for example, n-butyl 4,4-di(t-butyl peroxy) valerate, 1,1-di(t-butyl peroxy) 3,3,5-trimethyl cyclohexane, 1,1-di(t-butyl peroxy)cyclohexane, 1,1-di(t-amyl peroxy)cyclohexane, 2,2-di(t-butyl peroxy) butane, ethyl 3,3-di(t-butyl peroxy) butyrate and ethyl 3,3-di(t-amyl peroxy) butyrate, and combinations thereof.

10 Examples of suitable azo compounds include 2,2'-azobis(2,4-dimethylpentane nitrile), azobis-isobutyronitrile, 2,2'-azobis(isobutyronitrile), 2,2'-azobis(2,4-dimethyl valeronitrile), 2,2'-azobis(methyl butyronitrile), 1,1'-azobis(cyano cyclohexane), other similar known compounds, and combinations thereof.

15

Although any suitable initiator can be used, in embodiments the initiator may be an organic initiator that is soluble in any solvent present, but not soluble in water. For example, half-life/temperature characteristic plots for VAZO® 52 (2,2'-azobis(2,4-dimethylpentane nitrile), commercially available from E. I. du Pont de Nemours and Company, USA) shows a half-life greater than about 90 minutes at about 65° C. and less than about 20 minutes at about 80° C.

Where utilized, the crosslinker may be present in an amount of from about 0.5% by weight to about 20% by weight of the resin, in embodiments from about 1% by weight to about 10% by weight of the resin.

The crosslinker and amorphous resin may be combined for a sufficient time and at a sufficient temperature to form the crosslinked polyester gel. In embodiments, the crosslinker and amorphous resin may be heated to a temperature of from about 25° C. to about 99° C., in embodiments from about 30° C. to about 95° C., for a period of time of from about 1 minute to about 10 hours, in embodiments from about 5 minutes to about 5 hours, to form a crosslinked polyester resin or polyester gel suitable for use as a shell.

A single crosslinked polyester resin may be utilized as the shell or, in embodiments, a first crosslinked polyester resin may be combined with other resins to form a shell. For example, in embodiments, a crosslinked amorphous resin may be combined with additional amorphous resins to form a polyester gel shell. Multiple resins may be utilized in any suitable amounts. In embodiments, a first crosslinked amorphous polyester resin, for example a crosslinked amorphous resin of formula I above, may be present in an amount of from about 20 percent by weight to about 100 percent by weight of the total shell resin, in embodiments from about 30 percent by weight to about 90 percent by weight of the total shell resin. Thus, in embodiments, a second resin may be present in the shell resin in an amount of from about 0 percent by weight to about 80 percent by weight of the total shell resin, in embodiments from about 10 percent by weight to about 70 percent by weight of the shell resin.

The crosslinked shell resin may be applied to the aggregated particles by any method within the purview of those skilled in the art. In embodiments, the crosslinked polyester resin utilized to form the shell may be combined with a surfactant described above to form an emulsion. The emulsion possessing the crosslinked polyester resin may be combined with the aggregated particles described above so that the shell forms over the aggregated particles. Where the gel is in an emulsion, the gel emulsion may possess from about 1

percent solids by weight of the emulsion to about 80 percent solids by weight of the emulsion, in embodiments from about 5 percent solids by weight of the emulsion to about 60 percent solids by weight of the emulsion.

The formation of the shell over the aggregated particles may occur while heating to an elevated temperature in embodiments from about 35° C. to about 99° C., in embodiments from about 40° C. to about 80° C. The formation of the shell may take place for a period of time of from about 1 minute to about 5 hours, in embodiments from about 5 minutes to about 3 hours.

Utilizing the polyester gel to form a shell permits the use of high temperatures in formation of the shell and the subsequent coalescence of the toner particles, thereby expanding the process latitude while preventing the crystalline polyester from migrating to the surface of the toner particles.

#### Coalescence

Following aggregation to the desired particle size and application of the shell resin described above, the particles may then be coalesced to the desired final shape, the coalescence being achieved by, for example, heating the mixture to a suitable temperature. This temperature may, in embodiments, be from about 0° C. to about 50° C. higher than the onset melting point of the crystalline polyester resin utilized in the core, in other embodiments from about 5° C. to about 30° C. higher than the onset melting point of the crystalline polyester resin utilized in the core. For example, by utilizing the polyester gel in forming a shell as described above, in embodiments the temperature for coalescence may be from about 40° C. to about 99° C., in embodiments from about 50° C. to about 95° C. Higher or lower temperatures may be used, it being understood that the temperature is a function of the resins used.

Coalescence may also be carried out with stirring, for example at a speed of from about 50 rpm to about 1,000 rpm, in embodiments from about 100 rpm to about 600 rpm. Coalescence may be accomplished over a period of from about 1 minute to about 24 hours, in embodiments from about 5 minutes to about 10 hours.

After coalescence, the mixture may be cooled to room temperature, such as from about 20° C. to about 25° C. The cooling may be rapid or slow, as desired. A suitable cooling method may include introducing cold water to a jacket around the reactor. After cooling, the toner particles may be optionally washed with water, and then dried. Drying may be accomplished by any suitable method for drying including, for example, freeze-drying.

As the polyester resin utilized to form the shell is a gel, the shell resin may be able to prevent any crystalline resin in the core from migrating to the toner surface. In addition, the shell resin may be less compatible with the crystalline resin utilized in forming the core, which may result in a higher toner glass transition temperature (Tg). For example, toner particles having a shell of the present disclosure may have a glass transition temperature of from about 30° C. to about 80° C., in embodiments from about 35° C. to about 70° C. This higher Tg may, in embodiments, improve blocking and charging characteristics of the toner particles, including A-zone charging.

The gel utilized to form the shell may also have a high viscosity of from about 10,000,000 Poise to about 50,000,000 Poise, at coalescence temperature, for example from about 60° C. to about 90° C., in embodiments from about 65° C. to about 80° C., which may also play a role in preventing crystalline resin in the core from migrating to the toner surface, and thus improving A-zone charging. As the polyester resin utilized to form the shell is crosslinked and in the form of a

gel, the shell resin may be able to prevent any crystalline resin in the core from migrating to the toner surface.

Moreover, toners of the present disclosure having a gel in the shell may exhibit excellent document offset performance characteristics, as well as reduced peak gloss, in embodiments from about 20 Gardner gloss units (ggu) to about 100 ggu, in other embodiments from about 40 ggu to about 80 ggu, which may be desirable for reproduction of text and images, as some users object to high gloss and the differential which may occur between low gloss and high gloss. While not wishing to be bound by any theory, the reduction in peak gloss may be due to the higher viscosity of the toner compositions, which as noted above, may be due to the higher viscosity of the gel utilized in forming the shell. Toners of the present disclosure also have excellent crease MFT properties.

In embodiments, the polyester gel utilized to form the shell may be present in an amount of from about 2 percent by weight to about 40 percent by weight of the dry toner particles, in embodiments from about 5 percent by weight to about 35 percent by weight of the dry toner particles.

#### Additives

In embodiments, the toner particles may also contain other optional additives, as desired or required. For example, the toner may include positive or negative charge control agents, for example in an amount of from about 0.1 to about 10 percent by weight of the toner, in embodiments from about 1 to about 3 percent by weight of the toner. Examples of suitable charge control agents include quaternary ammonium compounds inclusive of alkyl pyridinium halides; bisulfates; alkyl pyridinium compounds, including those disclosed in U.S. Pat. No. 4,298,672, the disclosure of which is hereby incorporated by reference in its entirety; organic sulfate and sulfonate compositions, including those disclosed in U.S. Pat. No. 4,338,390, the disclosure of which is hereby incorporated by reference in its entirety; cetyl pyridinium tetrafluoroborates; distearyl dimethyl ammonium methyl sulfate; aluminum salts such as BONTRON E84™ or E88™ (Hodogaya Chemical); combinations thereof, and the like. Such charge control agents may be applied simultaneously with the shell resin described above or after application of the shell resin.

There can also be blended with the toner particles external additive particles including flow aid additives, which additives may be present on the surface of the toner particles. Examples of these additives include metal oxides such as titanium oxide, silicon oxide, tin oxide, mixtures thereof, and the like; colloidal and amorphous silicas, such as AEROSIL®, metal salts and metal salts of fatty acids inclusive of zinc stearate, aluminum oxides, cerium oxides, and mixtures thereof. Each of these external additives may be present in an amount of from about 0.1 percent by weight to about 5 percent by weight of the toner, in embodiments of from about 0.25 percent by weight to about 3 percent by weight of the toner. Suitable additives include those disclosed in U.S. Pat. Nos. 3,590,000, 3,800,588, and 6,214,507, the disclosures of each of which are hereby incorporated by reference in their entirety. Again, these additives may be applied simultaneously with the shell resin described above or after application of the shell resin.

In embodiments, toners of the present disclosure may be utilized as ultra low melt (ULM) toners. In embodiments, the dry toner particles having a shell of the present disclosure may, exclusive of external surface additives, have the following characteristics:

(1) Volume average diameter (also referred to as “volume average particle diameter”) of from about 3 to about 25  $\mu\text{m}$ , in embodiments from about 4 to about 15  $\mu\text{m}$ , in other embodiments from about 5 to about 12  $\mu\text{m}$ .

(2) Number Average Geometric Size Distribution (GSD<sub>n</sub>) and/or Volume Average Geometric Size Distribution (GSD<sub>v</sub>) of from about 1.05 to about 1.55, in embodiments from about 1.1 to about 1.4.

(3) Circularity of from about 0.93 to about 1, in embodiments from about 0.95 to about 0.99 (measured with, for example, a Sysmex FPIA 2100 analyzer).

The characteristics of the toner particles may be determined by any suitable technique and apparatus. Volume average particle diameter D<sub>50v</sub>, GSD<sub>v</sub>, and GSD<sub>n</sub> may be measured by means of a measuring instrument such as a Beckman Coulter Multisizer 3, operated in accordance with the manufacturer's instructions. Representative sampling may occur as follows: a small amount of toner sample, about 1 gram, may be obtained and filtered through a 25 micrometer screen, then put in isotonic solution to obtain a concentration of about 10%, with the sample then run in a Beckman Coulter Multisizer 3.

Toners produced in accordance with the present disclosure may possess excellent charging characteristics when exposed to extreme relative humidity (RH) conditions. The low-humidity zone (C zone) may be about 10° C./15% RH, while the high humidity zone (A zone) may be about 28° C./85% RH. Toners of the present disclosure may possess A zone charging of from about -3  $\mu$ C/g to about -35  $\mu$ C/g, in embodiments from about -4  $\mu$ C/g to about -30  $\mu$ C/g, a parent toner charge per mass ratio (Q/M) of from about -3  $\mu$ C/g to about -35  $\mu$ C/g, in embodiments from about -4  $\mu$ C/g to about -30  $\mu$ C/g, and a final triboelectric charge of from -10  $\mu$ C/g to about -45  $\mu$ C/g, in embodiments from about -12  $\mu$ C/g to about -40  $\mu$ C/g.

In accordance with the present disclosure, the charging of the toner particles may be enhanced, so less surface additives may be required, and the final toner charging may thus be higher to meet machine charging requirements.

#### Developers

The toner particles thus obtained may be formulated into a developer composition. The toner particles may be mixed with carrier particles to achieve a two-component developer composition. The toner concentration in the developer may be from about 1% to about 25% by weight of the total weight of the developer, in embodiments from about 2% to about 15% by weight of the total weight of the developer.

#### Carriers

Examples of carrier particles that can be utilized for mixing with the toner include those particles that are capable of triboelectrically obtaining a charge of opposite polarity to that of the toner particles. Illustrative examples of suitable carrier particles include granular zircon, granular silicon, glass, steel, nickel, ferrites, iron ferrites, silicon dioxide, and the like. Other carriers include those disclosed in U.S. Pat. Nos. 3,847,604, 4,937,166, and 4,935,326.

The selected carrier particles can be used with or without a coating. In embodiments, the carrier particles may include a core with a coating thereover which may be formed from a mixture of polymers that are not in close proximity thereto in the triboelectric series. The coating may include fluoropolymers, such as polyvinylidene fluoride resins, terpolymers of styrene, methyl methacrylate, and/or silanes, such as triethoxy silane, tetrafluoroethylenes, other known coatings and the like. For example, coatings containing polyvinylidene-fluoride, available, for example, as KYNAR 301F<sup>TM</sup>, and/or polymethylmethacrylate, for example having a weight average molecular weight of about 300,000 to about 350,000, such as commercially available from Soken, may be used. In embodiments, polyvinylidenefluoride and polymethylmethacrylate (PMMA) may be mixed in proportions of from about 30 to about 70 weight % to about 70 to about 30 weight %, in embodiments from about 40 to about 60 weight % to about 60 to about 40 weight %. The coating may have a

coating weight of, for example, from about 0.1 to about 5% by weight of the carrier, in embodiments from about 0.5 to about 2% by weight of the carrier.

In embodiments, PMMA may optionally be copolymerized with any desired comonomer, so long as the resulting copolymer retains a suitable particle size. Suitable comonomers can include monoalkyl, or dialkyl amines, such as a dimethylaminoethyl methacrylate, diethylaminoethyl methacrylate, diisopropylaminoethyl methacrylate, or t-butylaminoethyl methacrylate, and the like. The carrier particles may be prepared by mixing the carrier core with polymer in an amount from about 0.05 to about 10 percent by weight, in embodiments from about 0.01 percent to about 3 percent by weight, based on the weight of the coated carrier particles, until adherence thereof to the carrier core by mechanical impaction and/or electrostatic attraction.

Various effective suitable means can be used to apply the polymer to the surface of the carrier core particles, for example, cascade roll mixing, tumbling, milling, shaking, electrostatic powder cloud spraying, fluidized bed, electrostatic disc processing, electrostatic curtain, combinations thereof, and the like. The mixture of carrier core particles and polymer may then be heated to enable the polymer to melt and fuse to the carrier core particles. The coated carrier particles may then be cooled and thereafter classified to a desired particle size.

In embodiments, suitable carriers may include a steel core, for example of from about 25 to about 100  $\mu$ m in size, in embodiments from about 50 to about 75  $\mu$ m in size, coated with about 0.5% to about 10% by weight, in embodiments from about 0.7% to about 5% by weight, of a conductive polymer mixture including, for example, methylacrylate and carbon black using the process described in U.S. Pat. Nos. 5,236,629 and 5,330,874.

The carrier particles can be mixed with the toner particles in various suitable combinations. The concentrations are may be from about 1% to about 20% by weight of the toner composition. However, different toner and carrier percentages may be used to achieve a developer composition with desired characteristics.

#### Imaging

The toners can be utilized for electrostatographic or xerographic processes, including those disclosed in U.S. Pat. No. 4,295,990, the disclosure of which is hereby incorporated by reference in its entirety. In embodiments, any known type of image development system may be used in an image developing device, including, for example, magnetic brush development, jumping single-component development, hybrid scavengerless development (HSD), and the like. These and similar development systems are within the purview of those skilled in the art.

Imaging processes include, for example, preparing an image with a xerographic device including a charging component, an imaging component, a photoconductive component, a developing component, a transfer component, and a fusing component. In embodiments, the development component may include a developer prepared by mixing a carrier with a toner composition described herein. The xerographic device may include a high speed printer, a black and white high speed printer, a color printer, and the like.

Once the image is formed with toners/developers via a suitable image development method such as any one of the aforementioned methods, the image may then be transferred to an image receiving medium such as paper and the like. In embodiments, the toners may be used in developing an image in an image-developing device utilizing a fuser roll member. Fuser roll members are contact fusing devices that are within the purview of those skilled in the art, in which heat and pressure from the roll may be used to fuse the toner to the image-receiving medium. In embodiments, the fuser member

may be heated to a temperature above the fusing temperature of the toner, for example to temperatures of from about 70° C. to about 160° C., in embodiments from about 80° C. to about 150° C., in other embodiments from about 90° C. to about 140° C., after or during melting onto the image receiving substrate.

In embodiments where the toner resin is crosslinkable, such crosslinking may be accomplished in any suitable manner. For example, the toner resin may be crosslinked during fusing of the toner to the substrate where the toner resin is crosslinkable at the fusing temperature. Crosslinking also may be effected by heating the fused image to a temperature at which the toner resin will be crosslinked, for example in a post-fusing operation. In embodiments, crosslinking may be effected at temperatures of from about 160° C. or less, in embodiments from about 70° C. to about 160° C., in other embodiments from about 80° C. to about 140° C.

The following Examples are being submitted to illustrate embodiments of the present disclosure. These Examples are intended to be illustrative only and are not intended to limit the scope of the present disclosure. Also, parts and percentages are by weight unless otherwise indicated. As used herein, "room temperature" refers to a temperature of from about 20° C. to about 25° C.

## EXAMPLES

### Comparative Example 1

About 397.99 grams of a linear amorphous resin in an emulsion (about 17.03 weight % resin) was added to a 2 liter beaker. The linear amorphous resin was of the following formula:



wherein m was from about 5 to about 1000 and was produced following the procedures described in U.S. Pat. No. 6,063,827, the disclosure of which is hereby incorporated by reference in its entirety. About 74.27 grams of an unsaturated crystalline polyester ("UCPE") resin composed of ethylene glycol and a mixture of dodecanedioic acid and fumaric acid co-monomers with the following formula:



wherein b is from 5 to 2000 and d is from 5 to 2000 in an emulsion (about 19.98 weight % resin), synthesized following the procedures described in U.S. Patent Application Publication No. 2006/0222991, the disclosure of which is hereby incorporated by reference in its entirety, and about 29.24 grams of a cyan pigment, Pigment Blue 15:3, (about 17

weight %) was added to the beaker. About 36 grams of Al<sub>2</sub>(SO<sub>4</sub>)<sub>3</sub> (about 1 weight %) was added as flocculent under homogenization by mixing the mixture at about 3000 to 4000 rpm.

5 The mixture was subsequently transferred to a 2 liter Buchi reactor, and heated to about 45.9° C. for aggregation and mixed at a speed of about 750 rpm. The particle size was monitored with a Coulter Counter until the size of the particles reached an average volume particle size of about 6.83 10 µm with a Geometric Size Distribution ("GSD") of about 1.21.

About 198.29 grams of the above emulsion with the resin of formula I was then added to the particles to form a shell thereover, resulting in particles possessing a core/shell structure with an average particle size of about 8.33 µm, and a GSD of about 1.21.

15 Thereafter, the pH of the reaction slurry was increased to about 6.7 by adding NaOH followed by the addition of about 0.45 pph EDTA (based on dry toner) to stop, that is stop, the 20 toner growth. After stopping the toner growth, the reaction mixture was heated to about 69° C. and kept at that temperature for about 1 hour for coalescence.

The resulting toner particles had a final average volume 25 particle size of about 8.07, a GSD of about 1.22, and a circularity of about 0.976.

The toner slurry was then cooled to room temperature, separated by sieving (utilizing a 25 µm sieve) and filtered, followed by washing and freeze drying.

### Example 1

A gel latex was prepared as follows. About 125 grams of the amorphous propoxylated bisphenol A fumarate resin of

45 formula I as described in Comparative Example 1 above, with an acid number of about 17 as measured by titration with KOH, was combined with about 3.75 grams of VAZOR® 52 50 free radical thermal initiator (E. I. du Pont de Nemours and Company, USA) in a 2 liter beaker containing about 919 grams of ethyl acetate. The mixture was stirred at about 250 revolutions per minute (rpm) and heated to about 67° C. to 55 dissolve the resin and initiator in the ethyl acetate.

About 4.37 grams of sodium bicarbonate and about 1.34 55 grams (46.8 wt %) of DOWFAX™ 2A1, an alkyldiphenyloxide disulfonate (from The Dow Chemical Company, Midland, Mich.), were measured into a 4 liter Pyrex glass flask reactor containing about 708 grams of deionized water and heated to about 67° C. Homogenization of this heated water solution in 60 the 4 liter glass flask reactor occurred utilizing an IKA Ultra Turrax T50 homogenizer at about 4,000 revolutions per minute for about 30 minutes. The heated resin and initiator solution was then slowly poured into the water solution over a period of about 10 minutes. The homogenizer speed was 65 increased to about 10,000 revolutions per minute and homogenization continued for about 30 minutes. Upon completion of homogenization, the glass flask reactor and its contents

were placed in a heating mantle and connected to a distillation device. The mixture was stirred at about 400 revolutions per minute and the temperature of the mixture was increased to about 80° C. at about 1° C. per minute to distill off the ethyl acetate from the mixture. Stirring continued at about 80° C. for about 120 minutes followed by cooling at a rate of about 2° C. per minute until the mixture was at room temperature.

The amount of crosslinked portion of the gel was measured by a toluene solubility method, which was as follows. Approximately 40 mg of the above gel emulsion, which was first dried, was weighed out into a glass scintillation vial to which about 20 ml of toluene was added. The sample was shaken for about four hours on the low setting in a box shaker. The dissolution of the sample in toluene was followed by a vacuum filtration. The collecting membrane was dried under vacuum at about 65° C. for about four hours and weighed for % gel retained. About 6% of the gel produced above in Example 1 was determined to be crosslinked.

The product was screened through a 20 micron sieve and the pH was adjusted to about 7 with the addition of about 1 N sodium hydroxide. The resulting gel emulsion included about 32.72 percent by weight solids in water, and had a volume average diameter of about 153 nanometers as measured with a HONEYWELL MICROTAC® UPA150 particle size analyzer. The onset glass transition temperature was about 61.9° C. as measured by DSC.

#### Example 2

This Example produced toner particles possessing a core/ shell configuration, with about 28% by weight of a polyester gel from Example 1 in the shell.

About 296.34 grams of the linear amorphous resin of formula I as described in Comparative Example 1 above in an emulsion (about 17.02 weight % resin) was added to a 2 liter beaker. About 62.99 grams of the unsaturated crystalline polyester resin, depicted as formula II in Comparative Example 1 above, in an emulsion (about 17.53 weight % resin), and about 21.76 grams of a cyan pigment, Pigment Blue 15:3, (about 17 weight %) was added to the beaker. About 26.79 grams of Al<sub>2</sub>(SO<sub>4</sub>)<sub>3</sub> (about 1 weight %) was added as flocculent under homogenization by mixing the mixture at about 3000 to 4000 rpm.

The mixture was subsequently transferred to a 2 liter Buchi reactor, and heated to about 40° C. for aggregation and mixed at a speed of about 750 rpm. The particle size was monitored with a Coulter Counter until the size of the particles reached an average volume particle size of about of 7.42  $\mu$ m with a Geometric Size Distribution ("GSD") of about 1.23.

About 76.8 grams of the gel emulsion from Example 1 above was added as a shell, resulting in core-shell structured particles with an average particle size of about 8.96 microns, and a GSD of about 1.23.

Thereafter, the pH of the reaction slurry was increased to about 6.13 using NaOH followed by addition of 0.45 ppm EDTA (based on dry toner) to freeze, that is stop, the toner growth. After stopping the toner growth, the reaction mixture was heated to about 90° C. and kept at that temperature for about 0.5 hours for coalescence.

The resulting toner particles had a final particle size of about 8.24 microns and a GSD of about 1.29 and a circularity of about 0.953.

The toner slurry was then cooled to room temperature, separated by sieving (utilizing a 25  $\mu$ m sieve) and filtered, followed by washing and freeze drying.

The rheology of the toners of this Example and the control toner of Comparative Example 1 above was determined by

dynamic temperature step method using a Dynamic Stress Rheometer SR 5000, made by Maple Instruments Inc., following the manufacturer's instructions. The results are set forth in FIG. 1. As can be seen in FIG. 1, the viscosity of the toner of the present disclosure, possessing a polyester gel in the shell, was much higher than that of the toner of Comparative Example 1 (which had a polyester, but not a polyester gel in the shell), at higher temperatures (from about 130° C. to about 160° C.). The increased viscosity at this temperature range enabled reduction of peak gloss during fusing.

Fusing characteristics of the toners produced in Comparative Example 1 and the Examples were also determined by crease area, minimum fixing temperature, gloss, document offset, and vinyl offset testing.

#### Crease Area

The toner image displays mechanical properties such as crease, as determined by creasing a section of the substrate such as paper with a toned image thereon and quantifying the degree to which the toner in the crease separates from the paper. A good crease resistance may be considered a value of less than 1 mm, where the average width of the creased image is measured by printing an image on paper, followed by (a) folding inwards the printed area of the image, (b) passing over the folded image a standard TEFLON coated copper roll weighing about 860 grams, (c) unfolding the paper and wiping the loose ink from the creased imaged surface with a cotton swab, and (d) measuring the average width of the ink free creased area with an image analyzer. The crease value can also be reported in terms of area, especially when the image is sufficiently hard to break unevenly on creasing; measured in terms of area, crease values of 100 millimeters correspond to about 1 mm in width. Further, the images exhibit fracture coefficients, for example of greater than unity. From the image analysis of the creased area, it is possible to determine whether the image shows a small single crack line or is more brittle and easily cracked. A single crack line in the creased area provides a fracture coefficient of unity while a highly cracked crease exhibits a fracture coefficient of greater than unity. The greater the cracking, the greater the fracture coefficient. Toners exhibiting acceptable mechanical properties, which are suitable for office documents, may be obtained by utilizing the aforementioned thermoplastic resins. However, there is also a need for digital xerographic applications for flexible packaging on various substrates. For flexible packaging applications, the toner materials must meet very demanding requirements such as being able to withstand the high temperature conditions to which they are exposed in the packaging process and enabling hot pressure-resistance of the images. Other applications, such as books and manuals, require that the image does not document offset onto the adjacent image. These additional requirements require alternate resin systems, for example that provide thermoset properties such that a crosslinked resin results after fusing or post-fusing on the toner image.

#### Minimum Fixing Temperature

The Minimum Fixing Temperature (MFT) measurement involves folding an image on paper fused at a specific temperature, and rolling a standard weight across the fold. The print can also be folded using a commercially available folder such as the Duplo D-590 paper folder. The folded image is then unfolded and analyzed under the microscope and assessed a numerical grade based on the amount of crease showing in the fold. This procedure is repeated at various temperatures until the minimum fusing temperature (showing very little crease) is obtained.

## Gloss

Print gloss (Gardner gloss units or "ggu") was measured using a 75° BYK Gardner gloss meter for toner images that had been fused at a fuser roll temperature range of about 120° C. to about 210° C. (sample gloss was dependent on the toner, the toner mass per unit area, the paper substrate, the fuser roll, and fuser roll temperature).

## Document Offset

A standard document offset mapping procedure was performed as follows. Five centimeter (cm) by five cm test samples were cut from the prints taking care that when the sheets are placed face to face, they provide both toner to toner and toner to paper contact. A sandwich of toner to toner and toner to paper was placed on a clean glass plate. A glass slide was placed on the top of the samples and then a weight comprising a 2000 gram mass was placed on top of the glass slide. The glass plate was then inserted into an environmental chamber at a temperature of 60° C. where the relative humidity was kept constant at 50%. After 7 days, the samples were removed from the chamber and allowed to cool to room temperature before the weight was removed. The removed samples were then carefully peeled apart. The peeled samples were mounted onto a sample sheet and then visually rated with a Document Offset Grade from 5.0 to 1.0, wherein a lower grade indicates progressively more toner offset, ranging from none (5.0) to severe (1.0). Grade 5.0 indicates no toner offset and no adhesion of one sheet to the other. Grade 4.5 indicates noticeable adhesion, but no toner offset. Grade 4 indicates that a very small amount of toner offsets to the other sheet. Grade 3 indicates that less than 1/3 of the toner image offsets to the other sheet, while Grade 1.0 indicates that more than 1/2 of the toner image offsets to the other sheet. In general, an evaluation of greater than or equal to 3.0 is considered the minimum acceptable offset, and an evaluation of greater than or equal to 4.0 is desirable.

## Vinyl Offset

Vinyl offset was evaluated as follows. Toner images were covered with a piece of standard vinyl (32% dioctyl phthalate Plasticizer), placed between glass plates, loaded with a 250 gram weight, and placed in an environmental oven at a pressure of 10 g/cm<sup>2</sup>, 50° C. and 50% relative humidity (RH). After about 24 hours, the samples were removed from the oven and allowed to cool to room temperature. The vinyl and toner image were carefully peeled apart, and evaluated with reference to a vinyl offset evaluation rating procedure as described above for document offset wherein Grades 5.0 to 1.0 indicate progressively higher amounts of toner offset onto the vinyl, from none (5.0) to severe (1.0). Grade 5.0 indicates no visible toner offset onto the vinyl and no disruption of the image gloss. Grade 4.5 indicates no toner offset, but some disruption of image gloss. An evaluation of greater than or equal to 4.0 is considered an acceptable grade.

The results are summarized below in Table 1.

TABLE 1

| Goal                 | Comparative Example 1 | Example 2 |
|----------------------|-----------------------|-----------|
| DCX+ (90 gsm) paper  |                       |           |
| Cold Offset          | 113                   | 125       |
| Hot Offset           | >210                  | >210      |
| T <sub>G40</sub>     | ≤175° C.              | N/A       |
| Gloss @ MFT          | 40 ggu                | 38.0      |
| Gloss @ 185° C.      | ≥40                   | 72.5      |
| Peak Gloss           | ≥50                   | 72.6      |
| MFT <sub>CA-85</sub> | ≤169° C.              | 140       |
|                      |                       | 157       |

TABLE 1-continued

|    | Goal                                        | Comparative Example 1 | Example 2              |
|----|---------------------------------------------|-----------------------|------------------------|
| 5  | AMFT <sub>CA-85</sub>                       | Gloss 40 & CA = 85    | -34 -22                |
|    | MFT/AMFT                                    |                       | 142/34 N/A             |
|    | FC <sub>CA-85</sub>                         |                       | 4.34 4.55              |
|    | Document Offset (Toner-Toner) SIR (rmasLA)  | ≥1                    | 1.00 (15.1) 1.50 (4.7) |
| 10 | Document Offset (Toner-Paper) SIR (% toner) | ≥1                    | 1.00 (1.5) 1.25 (2.1)  |
|    | DC EG (120 gsm) paper                       |                       |                        |
|    | T <sub>G40</sub>                            | ≤175° C. 40 ggu       | 141 196                |
|    | Gloss @ MFT                                 |                       | 31.5 22.2              |
| 15 | Gloss @ 185° C.                             | ≥40                   | 80.2 33.8              |
|    | Peak Gloss                                  | ≥50                   | 94.1 48.9              |
|    | MFT <sub>CA-85</sub>                        | ≤169° C.              | 137 162                |
|    | AMFT <sub>CA-85</sub>                       |                       | -34 -20                |

MFT = Minimum fixing temperature (minimum temperature at which acceptable adhesion of the toner to the support medium occurs)

DCX = Uncoated Xerox paper

DCEG = Coated Xerox paper

gsm = grams per square meter

CA = crease area

T<sub>G40</sub> = Fusing temperature to reach 40 gloss unit

25 As can be seen from the above data in Table 1, the fusing results demonstrated that image gloss was dramatically reduced with the polyester gel in the toner shell, while still meeting crease MFT specifications.

30 Scanning Electron Micrograph (SEM) images were obtained. The SEM images of the toner containing polyester gel in shell produced in this Example 2, which was coalesced at 90° C., showed that the high viscosity shell prevented the 35 crystalline polyester in the core from migrating to the surface of the toner particles, even though the coalescence temperature was much higher than the melting point of crystalline polyester (about 81° C.). In contrast, SEM images of the 40 control toner of Comparative Example 1, which had a polyester in its shell that was not cross-linked, demonstrated that coalescence had to be conducted at a temperature much lower than the melting point of the crystalline polyester, to prevent the crystalline polyester from melting or coming to the toner surface.

45 Charging characteristics of the toner of the present disclosure with gel in the shell and the toner of Comparative Example 1 (no gel) were also determined. The results are set forth in FIG. 2, which compares the charging of the toner of the present disclosure with the toner of Comparative Example 1 (without the gel latex) in both A-zone and C-zone (in FIG. 2, Q/m is charge, AZ is A-zone, CZ is C-zone, 5M is 5 minutes, and 60M is 60 minutes). As can be seen in FIG. 2, the 50 addition of polyester gel dramatically increased toner charging in A-zone and C-zone compared with the toner of Comparative Example 1 (without gel), which shows that adding a gel to the toner shell as disclosed herein was much better at preventing the crystalline polyester in the core from migrating to the toner particle surface, compared with the control shell that was not a gel, regardless of the coalescence temperature.

55 It will be appreciated that various of the above-disclosed and other features and functions, or alternatives thereof, may be desirably combined into many other different systems or applications. Also that various presently unforeseen or unanticipated alternatives, modifications, variations or improve-

ments therein may be subsequently made by those skilled in the art which are also intended to be encompassed by the following claims. Unless specifically recited in a claim, steps or components of claims should not be implied or imported from the specification or any other claims as to any particular order, number, position, size, shape, angle, color, or material.

The invention claimed is:

1. An emulsion aggregation toner comprising:

a core particle comprising at least one amorphous polyester resin, at least one crystalline polyester resin, and one or more optional ingredients selected from the group consisting of an optional colorant, an optional wax and combinations thereof; and

a partially crosslinked polyester shell resin encapsulating aggregated core particles comprising at least one amorphous resin selected from the group consisting of poly(propoxylated bisphenol co-fumarate), poly(ethoxylated bisphenol co-fumarate), poly(butyloxylated bisphenol co-fumarate), poly(co-propoxylated bisphenol co-ethoxylated bisphenol co-fumarate), poly(1,2-propylene fumarate), poly(propoxylated bisphenol co-maleate), poly(ethoxylated bisphenol co-maleate), poly(butyloxylated bisphenol co-maleate), poly(co-propoxylated bisphenol co-ethoxylated bisphenol co-maleate), poly(1,2-propylene maleate), poly(propoxylated bisphenol co-itaconate), poly(ethoxylated bisphenol co-itaconate), poly(butyloxylated bisphenol co-itaconate), poly(co-propoxylated bisphenol co-ethoxylated bisphenol co-itaconate), poly(1,2-propylene itaconate), and combinations thereof, wherein about 5 wt % to about 35 wt % of the amorphous resin is crosslinked,

wherein the viscosity of the shell is greater than the viscosity of the core, and wherein the toner exhibits a viscosity plateau at higher temperatures as compared to a toner without said polyester gel in the shell, and gloss of said toner is from about 20 ggu to about 100 ggu.

2. The toner according to claim 1, wherein the at least one amorphous resin of the core comprises a polyester selected from the group consisting of poly(propoxylated bisphenol co-fumarate), poly(ethoxylated bisphenol co-fumarate), poly(butyloxylated bisphenol co-fumarate), poly(co-propoxylated bisphenol co-ethoxylated bisphenol co-fumarate), poly(1,2-propylene fumarate), poly(propoxylated bisphenol co-maleate), poly(ethoxylated bisphenol co-maleate), poly(butyloxylated bisphenol co-maleate), poly(co-propoxylated bisphenol co-ethoxylated bisphenol co-maleate), poly(1,2-propylene maleate), poly(propoxylated bisphenol co-itaconate), poly(ethoxylated bisphenol co-itaconate), poly(butyloxylated bisphenol co-itaconate), poly(co-propoxylated bisphenol co-ethoxylated bisphenol co-itaconate), poly(1,2-propylene itaconate), and combinations thereof, and wherein

the amorphous resin of the core and the amorphous resin of the shell may be the same or different.

3. The toner according to claim 1, wherein the at least one crystalline resin comprises a polyester selected from the group consisting of poly(ethylene-adipate), poly(propylene-adipate), poly(butylene-adipate), poly(pentylene-adipate), poly(hexylene-adipate), poly(octylene-adipate), poly(ethylene-succinate), poly(propylene-succinate), poly(butylene-succinate), poly(pentylene-succinate), poly(hexylene-succinate), poly(octylene-succinate), poly(ethylene-sebacate), poly(propylene-sebacate), poly(butylene-sebacate), poly(pentylene-sebacate), poly(hexylene-sebacate), poly(octylene-sebacate), alkali copoly(5-sulfoisophthaloyl)-copoly(ethylene-adipate), alkali copoly(5-sulfoisophthaloyl)-copoly(propylene-adipate), alkali copoly(5-sulfoisophthaloyl)-copoly(butylene-adipate), alkali copoly(5-sulfoisophthaloyl)-copoly(pentylene-adipate), alkali copoly(5-sulfoisophthaloyl)-copoly(hexylene-adipate), alkali copoly(5-sulfoisophthaloyl)-copoly(octylene-adipate), alkali copoly(5-sulfoisophthaloyl)-copoly(ethylene-adipate), alkali copoly(5-sulfoisophthaloyl)-copoly(propylene-adipate), alkali copoly(5-sulfoisophthaloyl)-copoly(ethylene-adipate), alkali copoly(5-sulfoisophthaloyl)-copoly(ethylene-adipate), alkali copoly(5-sulfoisophthaloyl)-copoly(propylene-adipate), alkali copoly(5-sulfoisophthaloyl)-copoly(hexylene-adipate), alkali copoly(5-sulfoisophthaloyl)-copoly(octylene-adipate), alkali copoly(5-sulfoisophthaloyl)-copoly(ethylene-succinate), alkali copoly(5-sulfoisophthaloyl)-copoly(propylene-succinate), alkali copoly(5-sulfoisophthaloyl)-copoly(butylene-succinate), alkali copoly(5-sulfoisophthaloyl)-copoly(pentylene-succinate), alkali copoly(5-sulfoisophthaloyl)-copoly(hexylene-succinate), alkali copoly(5-sulfoisophthaloyl)-copoly(ethylene-sebacate), alkali copoly(5-sulfoisophthaloyl)-copoly(butylene-sebacate), alkali copoly(5-sulfoisophthaloyl)-copoly(pentylene-sebacate), alkali copoly(5-sulfoisophthaloyl)-copoly(hexylene-sebacate), alkali copoly(5-sulfoisophthaloyl)-copoly(ethylene-adipate), alkali copoly(5-sulfoisophthaloyl)-copoly(butylene-adipate), alkali copoly(5-sulfoisophthaloyl)-copoly(ethylene-adipate), alkali copoly(5-sulfoisophthaloyl)-copoly(propylene-adipate), alkali copoly(5-sulfoisophthaloyl)-copoly(butylene-adipate), alkali copoly(5-sulfoisophthaloyl)-copoly(pentylene-adipate), alkali copoly(5-sulfoisophthaloyl)-copoly(hexylene-adipate), and poly(octylene-adipate),

wherein alkali comprises a metal selected from the group consisting of sodium, lithium and potassium.

4. The toner according to claim 1, wherein the at least one amorphous resin of the shell comprises a poly(propoxylated bisphenol A co-fumarate) resin of the formula:



wherein  $m$  may be from about 5 to about 1000.

5. The toner according to claim 1, wherein the core has a viscosity of from about 10 Poise to about  $1 \times 10^6$  Poise, said shell has a viscosity of from about  $1 \times 10^7$  Poise to about  $5 \times 10^7$  Poise or both.

6. The toner according to claim 1, wherein the at least one crystalline resin is of the formula:



wherein  $b$  is from 5 to 2000 and  $d$  is from 5 to 2000.

7. The toner according to claim 1, wherein the colorant comprises dyes, pigments, combinations of dyes, combinations of pigments, and combinations of dyes and pigments, in an amount of from about 0.1 to about 35 percent by weight of the toner.

8. The toner according to claim 1, wherein the wax is selected from the group consisting of polyolefins, carnauba wax, rice wax, candelilla wax, sumacs wax, jojoba oil, beeswax, niontan wax, ozokerite, ceresin, paraffin wax, microcristalline wax, Fischer-Tropsch wax, stearyl stearate, behenyl behenate, butyl stearate, propyl oleate, glyceride monostearate, glyceride distearate, pentaerythritol tetra behenate, dietyleneglycol monostearate, dipropylene glycol distearate, diglyceryl distearate, triglyceryl tetra stearate, sorbitan monostearate, cholesterol stearate, and combinations thereof, present in an amount from about 1 weight percent to about 25 weight percent of the toner.

9. The toner according to claim 1, wherein the toner is of a size of from about 3 to about 25  $\mu\text{m}$ , possesses a circularity of from about 0.93 to about 1 or possesses a parent toner charge per mass ratio of from about  $-3 \mu\text{C/g}$  to about  $-35 \mu\text{C/g}$ .

10. The toner according to claim 1, wherein the at last one amorphous resin in the core comprises a polyester gel.

**11. An emulsion aggregation toner comprising:**

11.1 an emulsion aggregation toner comprising:  
a core particle comprising at least one amorphous polyester resin, at least one crystalline polyester resin, and one or more optional ingredients selected from the group consisting of an optional colorant, an optional wax, and combinations thereof; and

a partially crosslinked polyester shell resin encapsulating aggregated core particles comprising at least one amorphous resin selected from the group consisting of poly(propoxylated bisphenol co-fumarate), poly(ethoxylated bisphenol co-ftimarate), poly(butyloxylated bisphenol co-fumarate), poly(co-propoxylated bisphenol co-ethoxylated bisphenol co-fumarate), poly(1,2-propylene fumarate), poly(propoxylated bisphenol comaleate), poly(ethoxylated bisphenol co-maleate), poly(butyloxylated bisphenol co-maleate), poly(co-propoxylated bisphenol co-ethoxylated bisphenol co-maleate), poly(1,2-propylene maleate), poly(propoxylated bisphenol co-itaconate), poly(ethoxylated bisphenol co-itaconate), poly(butyloxylated bisphenol co-itaconate), poly(co-propoxylated bisphenol co-ethoxylated bisphenol co-itaconate), poly(1,2-propylene itaconate), and combinations thereof, wherein about 5 wt % to about 35 wt % of the amorphous resin is crosslinked and the shell resin prevents the crystalline resin in the core particle from migrating to the toner particle surface, wherein the a viscosity of the shell is greater than the viscosity of the core, and wherein the toner exhibits a

viscosity plateau at higher temperatures as compared to a toner without said polyester gel in the shell, and gloss of said toner is from about 20 ggu to about 100 ggu.

12. The toner according to claim 11, wherein the at least one crystalline resin comprises a polyester selected from the group consisting of poly(ethylene-adipate), poly(propylene-adipate), poly(butylene-adipate), poly(pentylene-adipate), poly(hexylene-adipate), poly(octylene-adipate), poly(ethylene-succinate), poly(propylene-succinate), poly(butylene-succinate), poly(pentylene-succinate), poly(hexylene-succinate), poly(octylene-succinate), poly(ethylene-sebacate), poly(propylene-sebacate), poly(butylene-sebacate), poly(pentylene-sebacate), poly(hexylene-sebacate), poly(octylene-sebacate), alkali copoly(5-sulfoisophthaloyl)-copolymers (ethylene-adipate), alkali copoly(5-sulfoisophthaloyl)-copolymers (propylene-adipate), alkali copoly(5-sulfoisophthaloyl)-copolymers (butylene-adipate), alkali copoly(5-sulfo-isophthaloyl)-copolymers (pentylene-adipate), alkali copoly(5-sulfo-isophthaloyl)-copolymers (hexylene-adipate), alkali copoly(5-sulfo-isophthaloyl)-copolymers (octylene-adipate), alkali copoly(5-sulfo-isophthaloyl)-copolymers (ethylene-succinate), alkali copoly(5-sulfoisophthaloyl)-copolymers (propylene-succinate), alkali copoly(5-sulfoisophthaloyl)-copolymers (butylenes-succinate), alkali copoly(5-sulfoisophthaloyl)-copolymers (pentylene-succinate), alkali copoly(5-sulfoisophthaloyl)-copolymers (hexylene-succinate), alkali copoly(5-sulfoisophthaloyl)-copolymers (octylene-succinate), alkali copoly(5-sulfo-isophthaloyl)-copolymers (ethylene-sebacate), alkali copoly(5-sulfo-isophthaloyl)-copolymers (butylene-sebacate), alkali copoly(5-sulfo-isophthaloyl)-copolymers (pentylene-sebacate), alkali copoly(5-sulfo-isophthaloyl)-copolymers (hexylene-sebacate), alkali copoly(5-sulfo-isophthaloyl)-copolymers (octylene-sebacate), alkali copoly(5-sulfo-isophthaloyl)-copolymers (ethylene-adipate), alkali copoly(5-sulfo-isophthaloyl)-copolymers (propylene-adipate), alkali copoly(5-sulfo-isophthaloyl)-copolymers (butylene-adipate), alkali copoly(5-sulfo-isophthaloyl)-copolymers (pentylene-adipate), alkali copoly(5-sulfo-isophthaloyl)-copolymers (hexylene-adipate), alkali copoly(5-sulfo-isophthaloyl)-copolymers (octylene-adipate), and poly(5-sulfo-isophthaloyl)-copolymers (octylene-adipate).

wherein alkali comprises a metal selected from the group consisting of sodium, lithium and potassium.

13. The toner according to claim 11, wherein the colorant comprises dyes, pigments, combinations of dyes, combinations of pigments, and combinations of dyes and pigments, in an amount of from about 0.1 to about 35 percent by weight of the toner.

14. The toner according to claim 11, wherein the wax is selected from the group consisting of polyolefins, carnauba wax, rice wax, candelilla wax, sumacs wax, jojoba oil, beeswax, montan wax, ozokerite, ceresin, paraffin wax, microcrystalline wax, Fischer-Tropsch wax, stearyl stearate, behenyl behenate, butyl stearate, propyl oleate, glyceride monostearate, glyceride distearate, pentaerythritol tetra behenate, diethyleneglycol monostearate, dipropyleneglycol distearate, diglyceryl distearate, triglyceryl tetrastearate, sorbitan monostearate, cholesterol stearate, and combinations thereof present in an amount from about 1 weight percent to about 25 weight percent of the toner.

65 15. The toner according to claim 11, wherein the at least one amorphous resin of the shell comprises a poly(propoxy-  
lated bisphenol A co-fumarate) resin of the formula:



wherein m may be from about 5 to about 1000.

16. The toner according to claim 11, wherein the toner is of a size of from about 3 to about 25  $\mu\text{m}$ , possesses a circularity of from about 0.93 to about 1 or possesses a parent toner charge per mass ratio of from about  $-3 \mu\text{C/g}$  to about  $-35 \mu\text{C/g}$ .

17. The toner according to claim 11, wherein the core has a viscosity of from about 20 Poise to about  $1 \times 10^5$  Poise, and wherein said shell has a viscosity of from about  $1 \times 10^7$  Poise to about  $5 \times 10^7$  Poise.

18. The toner according to claim 11, wherein the at least one amorphous resin of the core comprises a polyester selected from the group consisting of poly(propoxylated bisphenol co-fumarate), poly(ethoxylated bisphenol co-fumarate), poly(butyloxylated bisphenol co-fumarate), poly(co-propoxylated bisphenol co-ethoxylated bisphenol co-fumarate), poly(1,2-propylene fumarate), poly(propoxylated bisphenol co-maleate), poly(ethoxylated bisphenol co-maleate), poly(butyloxylated bisphenol co-maleate), poly(co-propoxylated bisphenol co-ethoxylated bisphenol co-maleate), poly(1,2-propylene maleate), poly(propoxylated

15 bisphenol co-itaconate), poly(ethoxylated bisphenol co-itaconate), poly(butyloxylated bisphenol co-itaconate), poly(co-propoxylated bisphenol co-ethoxylated bisphenol co-itaconate), poly(1,2-propylene itaconate), and combinations thereof, and wherein the amorphous resin of the core and the amorphous resin of the shell may be the same or different.

19. The toner according to claim 11, wherein the at least one crystalline resin is of the formula:



wherein b is from 5 to 2000 and d is from 5 to 2000.

20. The toner according to claim 11, wherein the at least one amorphous resin in the core comprises a polyester gel.

\* \* \* \* \*